

## UNITED STATES PATENT OFFICE

2,250,998

## WAX SUPPRESSOR

Rene J. Narberes, Concord, and Frank Derbenwick, Martinez, Calif., assignors to Shell Development Company, San Francisco, Calif., a corporation of Delaware

No Drawing. Application December 1, 1939,  
Serial No. 307,083

6 Claims. (Cl. 252—32)

This invention relates to a process for preventing or delaying the formation of solid wax in hydrocarbon oils, particularly petroleum oils such as gas oils, lubricating oils, coal tar oils, shale oils, and the like at temperatures which are either above or below the pour point.

Hydrocarbon oils which contain waxy constituents often lose their lippidity because of the separation of particles of solid wax. This separated wax appears either in the form of a cloud within the oil or as a more or less crystalline precipitate which may remain dispersed throughout the oil. Frequently, the separated wax will collect on the walls of the container, especially near the surface of the oil, or will rise to the oil surface. Such separation of wax often occurs at temperatures which are substantially above the congealing temperature or pour point of the oil, with the result that small constrictions in a lubricating system may become obstructed. The lack of clarity is in itself undesirable, because of the unattractive appearance of the oil. This separation of solid wax is manifested both in the formation of clouds of dispersed more or less crystalline precipitates and in the formation of surface wax.

It is one object of our invention to provide a process for reducing, delaying or preventing the separation of such particles of wax by the addition of certain innocuous substances to the oil which are hereinafter referred to as "wax suppressors." Other objects of the invention will be apparent from a reading of this specification.

It has been found that the above stated objects can be realized by the addition to a wax-bearing oil of small quantities of mixtures of certain natural non-paraffinic waxes with viscous SO<sub>2</sub> soluble mineral oil fractions. While it is already known that cloud formation can be suppressed by the addition of natural waxes, it has been found that mixtures of these waxes with viscous SO<sub>2</sub> soluble mineral oil fractions are undoubtedly more effective for this purpose. The amount of the mixture required to obtain a certain result is less than the amount of other compounds to obtain the same result.

The waxes which fall within the scope of the present invention are at least in part saponifiable and are characterized by the large content of high molecular weight fatty acids and/or esters

of said fatty acids with mono- or poly-hydroxy alcohols, said acid or acid radical generally containing between ten and thirty-five carbon atoms. These waxes should preferably be of a relatively light color.

Natural waxes which may be mixed with viscous SO<sub>2</sub> soluble mineral oil fractions in accordance with the present invention are, in particular, white beeswax, yellow beeswax, spermaceti (cetaceum), wool wax, bayberry wax, candelilla wax, carnauba wax, Chinese wax, cocoa wax, cottonseed wax, Japan wax and montan wax. Other natural waxes may also be used, the specific waxes recited having been selected because of their availability at low cost as commercial waxes.

The term viscous SO<sub>2</sub> soluble mineral oil fractions is used herein to designate SO<sub>2</sub> soluble mineral oil fractions having a viscosity above 250 seconds Saybolt Universal at 210° F., and materials contained therein. Such fractions may be produced by extraction of viscous mineral oil distillates or residues with a naphthenic solvent such as furfural, phenol, liquid SO<sub>2</sub>, cresylic acid, beta-beta-dichlorethyl ether, etc.

A preferred form of our invention lies in the use of certain materials contained in viscous SO<sub>2</sub> soluble mineral oil fractions that are known as albino asphalts.

The most satisfactory results have been obtained with mixtures of albino asphalt with beeswax or montan wax, or with mixtures of albino asphalts with beeswax and carnauba wax, and with mixtures of beeswax and montan wax. These constitute a preferred embodiment of the present invention.

The term "albino asphalt" is used to designate certain normally solid or semi-solid translucent petroleum plastics which have been obtained by means set forth in the copending Anderson application, Serial No. 186,133, filed January 21, 1938, and the United States Patent No. 1,989,045 to Merrill, and the Bray patent, United States No. 2,029,288.

According to the Anderson application, translucent plastics may be produced from Mid-Continent (mixed base) oils which have been topped and de-asphalting by extracting the oil with a naphthenic solvent to produce a raffinate and an extract, and redistilling the extract to produce a semi-solid or solid plastic. When

Western (asphaltic base) oils are used, the raffinate produced with a naphthenic solvent such as  $\text{SO}_2$  is re-extracted with a stronger naphthenic solvent such as furfural to produce a secondary extract. This secondary extract contains the desired plastic and may be redistilled to the desired consistency. According to the Merrill patent, translucent petroleum plastics may be produced by extracting a Western petroleum asphalt-free oil with a naphthenic solvent and removing the lower boiling components from the extract by distillation. The albino asphalt need not be obtained from fractions produced by extraction. Thus, according to the Bray patent such plastics can be prepared by the distillation of high boiling cracked material free from asphaltenes.

Albino asphalts produced by the above processes fall into two general types, one of which is acetone soluble and has a lower penetration index than the other, which is substantially acetone insoluble in an equal volume of acetone at 77° F.

The waxes and the viscous  $\text{SO}_2$  soluble mineral oil fractions may be dissolved in the oil either singly or in combination with one another. The effective quantity of the wax suppressor mixture required for inhibiting wax formation in different oils varies with the different wax suppressor mixtures and also depends upon the quantity and nature of the hydrocarbon wax in the oil and upon the temperature to which the oil is to be cooled.

It has been found that the effective quantities usually lie between 0.005% and 1.0% though amounts up to about 1.5% may be used to reduce the cloud point.

It has also been found that the above-described mixtures are effective in reducing the pour point of hydrocarbon oils. When used for this purpose, somewhat larger quantities of suppressor agent are generally desirable, generally not exceeding 2%.

Such quantities of wax suppressors as are used in this invention to suppress the separation of wax, may have no significant effect upon the pour point of the oil, but have a marked effect in preventing or retarding the separation of solid wax. However, when used in larger concentration, these suppressor mixtures do exhibit pour point reducing properties. Many of these waxes may have their effectiveness increased by having their acid constituents, which are naturally present, saponified.

Thus, the beeswax may, for instance, be treated with lead carbonate, calcium oxide, magnesium oxide, zinc oxide, cadmium oxide, barium oxide or other bases to convert the acidic constituents into the corresponding metal soaps. The beeswax metal oxide or salt thus treated, when used in conjunction with viscous  $\text{SO}_2$  soluble mineral oil fractions, often has a greater power for suppressing wax than when only plain beeswax is used with the viscous  $\text{SO}_2$  soluble mineral oil fractions.

It is possible to use not only the ordinary viscous  $\text{SO}_2$  soluble mineral oil fractions, but also the hydrogenated fractions such as albino asphalts described in the copending application of Anderson, Serial No. 293,339, filed September 5, 1939.

The wax suppressor agents may be added to the oils at ordinary or at elevated temperatures. If the oil being treated contains particles of separated solvent paraffin wax, it is generally desirable to warm the oil to dissolve this paraffinic

wax prior to treatment. The time required for dissolving the suppressor agent can be decreased greatly by warming and agitating the mixtures.

In large scale operations it is often desirable to dissolve a large concentrated oil and suppressor agent solution to the main body of oil. Alternatively, the suppressor agents can be conveniently dissolved in the oil by placing fragments of the mixture of agents in a perforated container which is suspended in the oil.

To illustrate the use and effect of the present wax suppressor agents, the following examples are presented, it being understood that the present invention is not limited to the particular wax mixtures with viscous  $\text{SO}_2$  soluble mineral oil fractions, temperatures, concentrations, or details contained therein. While the mixtures of viscous  $\text{SO}_2$  soluble mineral oil fractions and wax may contain these components in various proportions, it is preferable to use mixtures containing these components between the limits of 1:9 and 9:1 albino asphalt to wax, and still more preferable to set the limits between 3:1 and 1:3.

#### Examples

A sample of a motor oil having a Saybolt Universal viscosity of 1000 seconds at 100° F. and a viscosity index of approximately 55 was placed in a 4 oz. oil sample bottle and allowed to stand in an ice box for 48 hours. After standing a heavy crystalline deposition of wax was observed at the sides of the bottle (side wax) and a flocculent suspension of more amorphous wax was noted in the body of the oil (body wax).

The above test was repeated on the same oil under the same conditions with the exception that 0.1% of a blend of 33% beeswax and 67% 13 penetration albino asphalt was added. After 48 hours the oil so treated remained perfectly bright with no trace of wax precipitate or surface wax.

A sample of a motor oil having a Saybolt Universal viscosity of 100 seconds at 210° F. was placed in a 4 oz. sample bottle and allowed to stand in an ice box for 72 hours. After standing a heavy crystalline deposition of wax was observed at the sides of the bottle (side wax) and a flocculent suspension of more amorphous wax was noted in the body of the oil (body wax).

The above test was repeated on the same oil and under the same conditions with the exception that 3% of a blend of 33% beeswax and 67% of an  $\text{SO}_2$  extract of 500 S. S. U. viscosity at 210° F. from a heavy bulk distillate was added. After 72 hours the oil so treated remained bright with no wax precipitate or body wax, and but a slight trace of side wax.

Further tests were carried out with different motor oils using varying proportions of wax suppressor mixture. The samples were placed in a 4 oz. oil sample bottle and held at 45° F. for 72 hours. Commercially available beeswax and a 13 penetration albino asphalt was used in the tests. The lube oil extract used was an  $\text{SO}_2$  extract of 500 S. S. U. viscosity at 210° F. from a heavy bulk distillate.

The appearance of the sample as to body wax and side wax was then visually observed and recorded on an arbitrary basis. 0 indicates no visible wax; 1 a small amount of visible wax; 2 a moderate amount of visible wax, and 3 a fairly heavy deposit of visible wax.

The results of these tests are tabulated below:

| Oil treated                                                       | Percent added                |              | Wax test rating |             |
|-------------------------------------------------------------------|------------------------------|--------------|-----------------|-------------|
|                                                                   | Percent<br>albino<br>asphalt | Bees-<br>wax | Side<br>wax     | Body<br>wax |
| Motor oil Saybolt Universal viscosity of 1,000 seconds at 100° F. | None                         | None         | 2               | 2           |
|                                                                   | 0.017                        | 0.008        | 1               | 1-          |
|                                                                   | 0.033                        | 0.017        | 1               | 0+          |
|                                                                   | 0.067                        | 0.033        | 1-              | 0           |
|                                                                   | 0.134                        | 0.066        | 0+              | 0           |
|                                                                   | 0.268                        | 0.132        | 0+              | 0           |
|                                                                   | 0.2                          | None         | 2               | 2+          |
|                                                                   | None                         | 0.017        | 0+              | 2           |
|                                                                   | None                         | 0.066        | 2               | 2           |
|                                                                   | None                         | None         | 3               | 3           |
|                                                                   | 0.017                        | 0.008        | 0+              | 0           |
|                                                                   | 0.033                        | 0.017        | 0+              | 0           |
|                                                                   | 0.067                        | 0.033        | 0               | 0           |
| Motor oil S. A. E. 40                                             | 0.025                        | None         | 0+              | 2           |
|                                                                   | 0.05                         | None         | 0+              | 2           |
|                                                                   | 0.10                         | None         | 1-              | 2           |
|                                                                   | None                         | 0.05         | 0+              | 2           |
|                                                                   | None                         | 0.10         | 0+              | 2+          |
|                                                                   | None                         | None         | 2               | 3           |
|                                                                   | 0.067                        | 0.033        | 0+              | 0           |
|                                                                   | 0.134                        | 0.066        | 0+              | 0           |
|                                                                   | 0.2                          | 0.1          | 1-              | 0+          |
|                                                                   | None                         | 0.033        | 2               | 0           |
| Motor oil Saybolt Universal viscosity of 100 seconds at 210° F.   | Heavy<br>tube oil<br>extract | Bees-<br>wax |                 |             |
|                                                                   | None                         | None         | 2               | 3           |
|                                                                   | 0.067                        | 0.033        | 1-              | 0+          |
|                                                                   | 0.2                          | 0.1          | 0+              | 0           |

Lubricating oils containing our wax suppressors may contain in addition other wax suppressors such as chlorinated naphthalenes, oxidation inhibitors, blooming agents, extreme pressure agents, wedging agents, reducing agents, corrosion inhibitors, and other compounding ingredients.

We claim as our invention:

1. A limpid normally liquid oil composition comprising a hydrocarbon oil containing paraffin wax in amount sufficient to impart an undesirably high cloud point to said oil in the absence of a wax suppressor, and dissolved therein in a quantity of less than .1% of a mixture of albino asphalt together with a natural at least partly saponifiable wax, said quantity being sufficient to suppress the separation of paraffin wax above the pour point of the hydrocarbon oil.

2. A limpid normally liquid oil composition comprising a hydrocarbon oil containing paraffin wax in amount sufficient to impart an undesirably high cloud point to said oil in the absence of a wax suppressor, and dissolved there-

in a quantity of less than .1% of a mixture of albino asphalt together with a natural at least partly saponifiable wax selected from the group consisting of beeswax, spermaceti, bayberry wax, candelilla wax, carnauba wax, cottonseed wax, Japan wax and montan wax, said quantity being sufficient to suppress the separation of paraffin wax above the pour point of the hydrocarbon oil.

5 3. A limpid normally liquid oil composition comprising a hydrocarbon oil containing paraffin wax in amount sufficient to impart an undesirably high cloud point to said oil in the absence of a wax suppressor, and dissolved therein 10 a quantity less than .1% of a mixture of albino asphalt with beeswax, said quantity being sufficient to suppress separation of paraffin wax above the pour point of the hydrocarbon oil.

15 4. A limpid normally liquid oil composition comprising a hydrocarbon oil containing paraffin wax in amount sufficient to impart an undesirably high cloud point to said oil in the absence of a wax suppressor, and dissolved therein 20 a quantity less than .1% of a mixture of hydro- 25 genated albino asphalt with beeswax, said quantity being sufficient to suppress separation of paraffin wax above the pour point of the hydrocarbon oil.

25 5. A limpid normally liquid oil composition comprising a hydrocarbon oil containing paraffin wax in amount sufficient to impart an undesirably high cloud point to said oil in the absence of a wax suppressor, and dissolved therein 30 a quantity less than .1% of a mixture of albino asphalt and beeswax and a substance from the group consisting of montan wax and carnauba wax, said quantity being sufficient to suppress separation of paraffin wax above the pour point of the hydrocarbon oil.

35 6. A limpid normally liquid oil composition comprising a hydrocarbon oil containing paraffin wax in amount sufficient to impart an undesirably high cloud point to said oil in the absence of a wax suppressor, and dissolved therein 45 a quantity less than .1% of a mixture of albino asphalt with a natural at least partly saponifiable wax containing metal soaps resulting from converting its fatty acid components to metal soaps, said quantity being sufficient to suppress the separation of paraffin wax from the hydrocarbon oil.

RENE J. NARBERES.  
FRANK DERBENWICK.